

1

3,692,515  
FERROUS ALLOYS AND ABRASION RESISTANT  
ARTICLES THEREOF

Stewart G. Fletcher and Walter T. Haswell, Jr., Latrobe, Pa., assignors to Latrobe Steel Company  
Continuation-in-part of application Ser. No. 429,621, Feb. 1, 1965. This application July 30, 1968, Ser. No. 748,631  
The portion of the term of the patent subsequent to Jan. 13, 1987, has been disclaimed  
Int. Cl. C22c 39/20

U.S. CL. 75—126 A

7 Claims

#### ABSTRACT OF THE DISCLOSURE

An abrasion resistant alloy stock material consisting essentially of carbon about 1% to 4.25%, said carbon being in excess of that necessary to impart a desired hard-ability, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium being combined with said excess carbon in a weight ratio of 4:1 and the vanadium with carbon in a weight ratio of about 4.2 (V—1):1, said stock material having been reduced by working at least about 5% in cross-section.

This application is a continuation-in-part of our co-pending application Ser. No. 429,621 filed Feb. 1, 1965, now abandoned.

This invention relates to ferrous alloys and abrasion resistant articles thereof and particularly to a low cost abrasion resistant alloy which has been worked. The search for steels having high abrasion resistance and low cost, together with satisfactory workability, has been a long and continuing one. Examples of uses for such steels are brick mold liners, tile dies, sand blast equipment, shot blast equipment and various forms of dies. Alloys generally available at a favorable cost are undesirably short-lived and less than satisfactory for abrasion-resisting purposes.

We have discovered an alloy having improved forgeability, workability and abrasion resistance over any alloys previously available to the metallurgical industry. Our invention provides an abrasion-resistant alloy in which carbon within certain limits, is added in excess of that necessary to give a desired hardening ability to the alloy together with vanadium and titanium in certain proportions and within certain limits such that the excess carbon equals

$$\frac{V-1}{4.2} + \frac{Ti}{4}$$

Considering only the essential elements of our alloy, the preferred analysis for most abrasion-resisting applications is:

|            | Percent |
|------------|---------|
| Carbon     | 2.9     |
| Silicon    | 0.4     |
| Manganese  | 0.4     |
| Chromium   | 12.5    |
| Molybdenum | 1.1     |
| Titanium   | 3       |

Balance substantially iron with residual impurities in ordinary amounts, said titanium being combined with carbon in a weight ratio of 4:1.

The composition of our alloy may, however, extend

2

over a relatively wide range and still retain its desirable properties of workability and abrasion-resistance. It may include alloying elements such as nickel, cobalt, tungsten and vanadium within certain limited amounts and proportions without detrimentally affecting the abrasion-resistance. Such wider range of composition may fall within the following limits:

|            |                         |
|------------|-------------------------|
| Carbon     | About 1 to about 4.25%. |
| Silicon    | About 1.5% maximum.     |
| Manganese  | Do.                     |
| Chromium   | About 10% to about 15%. |
| Molybdenum | Less than 2%.           |
| Titanium   | About 0.5 to about 5%.  |
| Tungsten   | Less than 3%.           |
| Nickel     | Do.                     |
| Cobalt     | Less than 5%.           |
| Vanadium   | Do.                     |
| Sulfur     | Up to 0.25%.            |

Balance substantially iron with residual impurities in ordinary amounts, said titanium being combined with carbon in a weight ratio of 4:1 and the vanadium with carbon in a weight ratio of 4.2 (V—1):1.

The expression "less than" followed by a percentage figure in this application, in the context of this application means that the particular element may be entirely absent or it may be present in an amount not to exceed the percentage concentration given. The presence of these elements is optional up to the amount specified in the ranges of composition given above.

The alloy is cast and preferably worked by forging, rolling or the like to reduce the cross section in an amount equal to at least about 5% of the original size. The alloy articles are preferably heat treated after working by tempering to achieve a desired tempered hardness. Tempering is preferably carried out at temperatures in the range 900–950° F. after austenitizing at a temperature in the range 1600–1950° F.

In order to illustrate the improved properties of our new alloy, several heats were made within the range of composition herein specified and compared with steels previously used for making brick liners and the like. The compositions appear in Table I. Each of the articles was formed by hammer forging to reduce the cross section about 40% and tempered at 900° F.

TABLE I

| Alloy             | C    | Cr    | W | Mo   | Ti   | V | Si   | Mn  | Ni | Co |
|-------------------|------|-------|---|------|------|---|------|-----|----|----|
| Invention<br>WR66 | 2.37 | 12.64 | — | 1.02 | 2.83 | — | 0.39 | .47 | —  | —  |
| Invention<br>WR67 | 2.7  | 12.83 | — | 1.03 | 2.98 | — | 0.43 | .49 | —  | —  |
| Prior art         | 2.4  | 12.75 | — | 1.1  | —    | 4 | 0.40 | .40 | —  | —  |

55 Abrasion tests were made, comparing these several alloys with the results which appear in Table II.

Table II

| Alloy:    | Percent abrasion |
|-----------|------------------|
| WR66      | 2.24             |
| WR67      | 3.02             |
| Prior art | 3.76             |

65 Careful comparison of the foregoing results shows the superiority of our alloy over the alloys now used for abrasion resistant purposes. Moreover, we have found that the compositions with titanium present are far more workable than like compositions in which vanadium has been completely substituted for titanium, so that titanium must appear as an essential ingredient at least in the minimum amount specified herein in order to attain the improved workability along with improved abrasion resistance which characterizes our invention.

While we have described and disclosed certain preferred embodiments of this invention, it will be understood that this invention may be otherwise embodied within the scope of the following claims.

We claim:

1. An abrasion resistant alloy stock material consisting essentially of carbon about 1% to 4.25%, said carbon being in excess of that necessary to give it a desired hardenability, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium and vanadium being combined with carbon in excess of that necessary to give a desired hardenability in proportions such that titanium is combined with a portion of said excess carbon in a weight ratio of 4:1 and the vanadium with the balance of said excess carbon in a weight ratio of about 4.2 (V-1):1, said stock material having been reduced by working at least about 5% in cross sectional area from its as cast condition.

2. A formed article made from a ferrous base metal comprising carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium and vanadium being combined with carbon in excess of that necessary to give a desired hardenability in proportions such that titanium is combined with a portion of said excess carbon in a weight ratio of 4:1 and the vanadium with the balance of said excess carbon in a weight ratio of 4.2 (V-1):1, said alloy being characterized by workability, castability, abrasion resistance and high impact resistance and having been formed by working the base metal to reduce its cross section at least 5%.

3. A formed article of manufacture made from a ferrous base metal alloy capable of being worked and cast to ultimate shape comprising carbon about 2.9%, silicon about 0.4%, manganese about 0.4%, chromium about 12.5%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium being combined with carbon in a weight ratio of 4:1, said alloy characterized by workability, castability, abrasion resistance and high resistance to impact, and having been formed by working the base metal to reduce its cross section at least 5%.

4. A shot blast liner formed of an alloy consisting essentially of carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium and vanadium being combined with carbon in excess of that necessary to give a desired hardenability in proportions such that titanium is combined with a portion of said excess carbon in a weight ratio of 4.2 (V-1):1 to titanium carbide and the vanadium with the balance of said excess carbon in a weight ratio of 4.2 (V-1):1 to form vanadium carbide, said alloy being characterized by workability, castability, abrasion resistance and high impact resistance and having been formed by working the base metal to reduce its cross section at least 5% in forming the liner.

5. A sand blast liner formed of an alloy consisting

essentially of carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium and vanadium being combined with carbon in excess of that necessary to give a desired hardenability in proportions such that titanium is combined with a portion of said excess carbon in a weight ratio of 4:1 to form titanium carbide and the vanadium with the balance of said excess carbon in a weight ratio of 4.2 (V-1):1 to form vanadium carbide, said alloy being characterized by workability, castability, abrasion resistance and high impact resistance and having been formed by working the base metal to reduce its cross section at least 5% in forming the liner.

6. A brick mold liner formed of an alloy consisting essentially of carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium and vanadium being combined with carbon in excess of that necessary to give a desired hardenability in proportions such that titanium is combined with a portion of said excess carbon in a weight ratio of 4:1 to form titanium carbide and the vanadium with the balance of said excess carbon in a weight ratio of 4.2 (V-1):1 to form vanadium carbide, said alloy being characterized by workability, castability, abrasion resistance and high impact resistance and having been formed by working the base metal to reduce its cross section at least 5% in forming the liner.

7. A ceramic tile die formed of an alloy consisting essentially of carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium less than about 5%, sulfur up to about 0.25% and the balance iron with residual impurities in ordinary amounts, said titanium and vanadium being combined with carbon in excess of that necessary to give a desired hardenability in proportions such that titanium is combined with a portion of said excess carbon in a weight ratio of 4:1 to form titanium carbide and the vanadium with the balance of said excess carbon in a weight ratio of 4.2 (V-1):1 to form vanadium carbide, said alloy being characterized by workability, castability, abrasion resistance and high impact resistance and having been formed by working the base metal to reduce its cross section at least 5% in forming the liner.

#### References Cited

#### UNITED STATES PATENTS

|           |         |         |       |          |
|-----------|---------|---------|-------|----------|
| 1,599,425 | 9/1926  | McGuire | ----- | 75—126   |
| 2,147,121 | 2/1939  | Emmons  | ----- | 75—126   |
| 2,575,218 | 11/1951 | Giles   | ----- | 75—126   |
| 3,231,709 | 1/1966  | Folley  | ----- | 75—126 X |
| 3,295,401 | 1/1967  | Rackoff | ----- | 75—126 X |

#### OTHER REFERENCES

Tool Steels, 3rd ed., 1962, published by American Society for Metals, Metals Park, Ohio, pp. 699—704 and 718.

HYLAND BIZOT, Primary Examiner

U.S. CL. X.R.

UNITED STATES PATENT OFFICE  
CERTIFICATE OF CORRECTION

Patent No. 3,692,515 Dated September 19, 1972

Inventor(s) Stewart G. Fletcher, et. al.

It is certified that error appears in the above-identified patent and that said Letters Patent are hereby corrected as shown below:

Column 3, claim 4, line 68, after "of" cancel "4.2 (V-1) :1 to" and insert -- 4:1 to form -- . Column 4, claim 5, line 8, "residul" should read -- residual -- .

Signed and sealed this 2nd day of January 1973.

(SEAL)  
Attest:

EDWARD M.FLETCHER,JR.  
Attesting Officer

ROBERT GOTTSCHALK  
Commissioner of Patents